# EUROPEAN PATENT SPECIFICATION

(11) **EP 1 325 166 B1**
(45) Date of publication and mention of the grant of the patent: **29.11.2006**
(21) Application number: 01973874.9
(22) Date of filing: 10.09.2001
(51) Int. Cl.: C22C 38/38

(54) **Layered surface coating on a substrate of stainless steel and process of producing it**
Geschichtete Oberflächenbeschichtung auf nichtrostendem Stahl und Verfahren zu deren Herstellung
Revêtement multicouches sur un substrat d'acier inoxydable et son procédé de fabrication

(30) Priority: 12.09.2000 US 659361; 12.09.2000 US 660084
(43) Date of publication of application: 09.07.2003
(73) Proprietor: Nova Chemicals (International) S.A., 1700 Fribourg (CH)
(72) Inventor: BENUM, Leslie, Wilfred, Red Deer, Alberta T4N 2B9 (CA); OBALLA, Michael, C., Cochrane, Alberta T4C 1A2 (CA); PETRONE, Sabino, Steven, Anthony, Edmonton, Alberta T5K 0T5 (CA)
(74) Representative: Watson, Robert James
(86) International application number: PCT/CA2001/001290
(87) International publication number: WO 2002/022905

(56) References cited:
- EP-A- 0 548 405
- GB-A- 2 159 542
- GB-A- 2 169 621
- US-A- 3 919 073
- US-A- 4 379 745
- US-A- 5 873 951
- US-A- 5 944 981
- DATABASE CA [Online] CHEMICAL ABSTRACTS SERVICE, COLUMBUS, OHIO, US; NIPPON STEEL CORP., JAPAN: "Ferritic stainless steels with high corrosion-resistance" retrieved from STN Database accession no. 94:107577 CA XP002196024 -& JP 55 141545 A (NIPPON STEEL CORP., JAPAN) 5 November 1980 (1980-11-05)
- PATENT ABSTRACTS OF JAPAN vol. 009, no. 153 (C-288), 27 June 1985 (1985-06-27) -& JP 60 029459 A (SUMITOMO KINZOKU KOGYO KK), 14 February 1985 (1985-02-14)

## Description

### TECHNICAL FIELD

The present invention relates to stainless steel having a high chrome content adapted to support a spinel, preferably overcoating chromia. The overcoated surface has superior chemical stability in coke-forming environments of at least 25°C higher than a surface without the spinel (e.g. the chromia). Such stainless steel may be used in a number of applications, particularly in the processing of hydrocarbons and in particular in pyrolysis processes such as the dehydrogenation of alkanes to olefins (e.g. ethane to ethylene or propane to propylene); reactor tubes for cracking hydrocarbons; or reactor tubes for steam cracking or reforming.

### BACKGROUND ART

It has been known for some time that the surface composition of a metal may have a significant impact on its utility. It has been known to treat steel to produce an iron oxide layer that is easily removed. It has also been known to treat steel to enhance its wear resistance. As far as Applicants are aware there is not a significant amount of art on selecting a steel composition to support an overcoat (preferably on chromia) to significantly reduce coking in hydrocarbon processing.

It is known that some steels (e.g. high chromium steels) will produce a chromia coating under certain conditions. It is predicted that chromia stability against coking is significantly reduced under conditions where the carbon activity is about 1 (e.g. with a deposit of a carbon or coke layer). For example at temperatures greater than about 950°C and at low oxygen partial pressures chromia starts to be converted to chromium carbides. Such carbide formation leading to volume expansion, embrittlement and possible spallation, thereby leaving the surface unprotected and reducing the coking resistance of the steel tubes. The present invention seeks to address this problem.

U.S. patent 3,864,093 issued February 4, 1975 to Wolfla (assigned to Union Carbide Corporation) teaches applying a coating of various metal oxides to a steel substrate. The oxides are incorporated into a matrix comprising at least 40 weight % of a metal selected from the group consisting of iron, cobalt, and nickel and from 10 to 40 weight % of aluminum, silicon and chromium. The balance of the matrix is one or more conventional metals used to impart mechanical strength and/or corrosion resistance. The oxides may be oxides or spinels. The patent teaches that the oxides should not be present in the matrix in a volume fraction greater than about 50%, otherwise the surface has insufficient ductility, impact resistance, and resistance to thermal fatigue. The reference does not teach overcoatings to protect chromia nor does it suggest the composition of a steel adapted to support such a coating.

U.S. patent 5,536,338 issued July 16, 1996 to Metivier et al. (assigned to Ascometal S.A.) teaches annealing carbon steels rich in chromium and manganese in an oxygen rich environment. The treatment results in a surface scale layer of iron oxides slightly enriched in chromium. This layer can easily be removed by pickling. Interestingly, there is a third sub-scale layer produced which is composed of spinels of Fe, Cr and Mn. This is opposite to the subject matter of the present patent.

U.S. patent 4,078,949 issued March 14, 1978 to Boggs et al. (assigned to U.S. Steel) is similar to U.S. patent 5,536,338 in that the final surface sought to be produced is an iron based spinel. This surface is easily subject to pickling and removing of slivers, scabs and other surface defects. Again this art teaches away from the subject matter of the present invention.

U.S. patent 5,630, 887 issued May 20, 1997 to Benum et al. (assigned to Novacor Chemicals Ltd. (now NOVA Chemicals Corporation)) teaches the treatment of stainless steel to produce a surface coating having a thickness from about 20 to 45 microns, comprising from 15 to 25 weight % of manganese and from about 60 to 75 weight % of chromium.

The reference is silent about the composition of the outer layer and the presence of a chromia layer. GB-A-2 159 542 discloses producing a layered surface on a substrate of stainless steel comprising 20% Cr, 33% Ni, 4% Mn and less than 1% of each of Si, Ti, Al by annealing the substrate at 950°C at first in a hydrogen atmosphere and then in an atmosphere of CO₂. A first interlayer of Cr₂O₃ having a thickness of 2-3 µm and an outer layer of Mn Cr₂O₄ having a thickness of 1-2 µm are formed. The layered surface coating protects the substrate from corrosion at elevated temperature.

### DISCLOSURE OF INVENTION

The present invention provides a layered surface on a stainless steel substrate as defined in claim 1. The outermost layer having a thickness from 2 to 5 microns comprises not less than 80 weight % of a spinel of the formula MnₓCr₃₋ₓO₄ wherein x is from 0.5 to 2, said stainless steel comprising at least 20 weight % of chromium, at least 1.0 weight % of manganese, less than 1.0 weight % of niobium, and less than 1.5 weight % of silicon.

The outermost layer on the intermediate layer comprising chromia of the formula Cr₂O₃ provides stability against carburizing or oxidation at temperatures at least a 25°C higher than said chromia. Said at least one intermediate layer comprises not less than 80 weight % of chromia of the formula Cr₂O₃. Said outermost layer having a thickness from 1 to 10 microns comprises not less than 80 weight % of a spinel of the formula MnₓCr₃₋ₓO₄ wherein x is from 0.5 to 2 and covering not less than 100% of the geometrical area defined by said at least one layer intermediate the outermost layer and the substrate.

In accordance with a further aspect of the present invention there is provided a process for treating a stainless steel which process is characterized in claim 11. The stainless steel of the substrate comprises at least 20 weight % of chromium, at least 1.0 weight % of manganese, less than 1.0 weight % of niobium, and less than 1.5 weight % of silicon. The process comprises:
(i) heating the stainless steel in a reducing atmosphere comprising from 50 to 100 weight % of hydrogen; from 0 to 50 of one or more inert gases at rate of 100°C to 150°C per hour to a temperature from 800°C to 1100°C;
(ii) then subjecting the stainless steel to an oxidizing environment having an oxidizing potential equivalent to a mixture of from 30 to 50 weight % of air and from 70 to 50 weight % of one or more inert gases at a temperature from 800°C to 1100°C for a period of time from 5 to 40 hours; and
(iii) cooling the resulting stainless steel to room temperature at a rate so as not to damage the surface on the stainless steel.

### BRIEF DESCRIPTION OF DRAWINGS

Figure 1 is an SEM micrograph of the spinel overcoating of the present invention (low magnification 7,500X) exemplifying the high surface coverage (e.g. not less than 95%).
Figure 2 is an SEM micrograph of the same spinel overlayer of the present invention (high magnification 25,000X) exemplifying high surface area (e.g., not less than 150% of the surface of the substrate).
Figure 3 is a metallographic cross-section (magnification 1,000X) of the present invention exemplifying the oxide coverage consisting of a chromia sub-scale with a spinel overcoating. The micrograph also shows the presence of discontinuous silica phase at the steel-oxide interface.
Figure 4 is a typical EDS spectrum of the present invention.
Figure 5 are X-ray diffraction spectra demonstrating the thermal stability of pure chromia powder (Cr₂O₃. bottom spectrum with no graphite) in the temperature range of 950-1050°C under a carbon activity of essentially one (a_{c} ≅ 1).
Figure 6 is a coil pressure drop (kPa) of individual long runs of H-141 and 9 typical runs of H-151.
Figure 7 is a quench exchanger pressure drop (kPa) of individual long runs of H-141 and 9 typical runs of H-151.

### BEST MODE FOR CARRYING OUT THE INVENTION

The stainless steel which is the subject matter of the present invention typically comprises from 20 to 50, preferably from 20 to 38 weight % of chromium and at least 1.0 weight %, up to 2.5 weight % preferably not more than 2 weight % of manganese. The stainless steel should contain less than 1.0, preferably less than 0.9 weight % of niobium and less than 1.5, preferably less than 1.4 weight % of silicon. The stainless steel further comprises from 25 to 50 weight % of nickel, from 1.0 to 2.5 weight % of manganese and less than 3 weight % of titanium and all other trace metals, and carbon in an amount of less than 0.75 weight. The steel comprises from about 25 to 50, preferably from about 30 to 45 weight % nickel and generally less than 1.4 weight % of silicon. The balance of the stainless steel is substantially iron.

The stainless steel part has a layered surface having a thickness of from 7 to 25 microns on a stainless steel substrate, said surface comprising an outermost layer and at least one layer intermediate the outermost layer and the substrate, said at least one layer intermediate the outermost layer and the substrate comprising not less than 80 weight % of chromia preferably of the formula Cr₂O₃ and said outermost layer (or overcoating layer) having a thickness from 2 to 5 microns comprising not less than 80 weight % of a spinel of the formula MnₓCr₃₋ₓO₄ wherein x is from 0.5 to 2 and covering essentially 100% of the geometrical area defined by said at least one layer intermediate the outermost layer and the substrate.

Intermediate the outer most layer or overcoating layer and the stainless steel substrate is at least one layer intermediate the outermost layer and the substrate comprising not less than 80, preferably greater than 95, most preferably greater than 99 weight % of chromia preferably of the formula Cr₂O₃. The chromia layer covers not less than 80, preferably not less than 95, most preferably not less than 99% of the geometric surface of a stainless steel which is exposed to a hydrocarbon feed stream (e.g. a hydrocarbon feed stream flowing over the outer surface of the stainless steel. The chromia layer is immediately (below) the outer spinel layer. The outermost spinel layer consists of crystallites that cover the chromia layer. That is, essentially 100% of the geometrical area of the chromia is overcoated with the spinel. The spinel crystallite structure effectively increases surface area relative to the geometrical area defined by the base steel alloy and the plate-like chromia layer. This increase in surface area afforded by the spinel crystallites is at least 50% and preferably 100% and most preferably 200% or greater of the surface area defined by the chromia (i.e. the surface of the spinel crystallites is greater than the surface area of the chromia plates). This enhancement of surface area is expected, among other things, to significantly increase heat transfer capability where it is a desirable property.

The spinel outer surface or over coating has a thickness from 2 to 5 microns and is selected from the group consisting of a spinel of the formula MnₓCr₃₋ₓO₄ wherein x is from 0.5 to 2; preferably x is from 0.8 to 1.2, most preferably x is 1 and the spinel has the formula MnCr₂O₄.

The overall surface layers have a thickness from 7 to 25 microns. The surface layers at least comprise the outer surface preferably having a thickness from 2 to 5 microns. The chromia layer generally has a thickness from 5 to 20, preferably from 7 to 15 microns. As noted above the spinel overcoats the chromia geometrical surface area. There may be very small portions of the surface which may only be chromia and do not have the spinel overlayer. In this sense the layered surface may be non-uniform. Preferably, the chromia layer underlies or is adjacent not less than 80, preferably not less than 95, most preferably not less than 99% of the spinel.

The spinel overlayer over the chromia provides stability against oxidation or carburization at temperature at least 25°C higher than that of the underlying chromia. In environments having a carbon activity of approximately 1, for example (without limiting the scope of this disclosure) in a steam cracker at a temperature from 900°C to 1050°C using a hydrocarbon feed stream (e.g. low reducing atmosphere) the spinel overcoating has a stability against carburization typically from 25°C to 50°C higher than that for the corresponding chromia. In an oxidizing atmosphere the spinel overcoat provides a stability against oxidation at temperatures from 25°C to 100°C higher than the corresponding chromia.

One method of producing the surface of the present invention is by treating the shaped stainless steel (i.e. part which may have been cold worked prior to treatment) in a process which might be characterized as a heat/soak/cool process. The process comprises:
(i) heating the stainless steel in a reducing atmosphere comprising from 50 to 100, preferably 60 to 100, weight % of hydrogen and from 0 to 50, preferably from 0 to 40 weight % of one or more inert gases at rate of 100°C to 150°C, preferably from 120°C to 150°C, per hour to a temperature from 800°C to 1100°C;
(ii) then subjecting the stainless steel to an oxidizing environment having an oxidizing potential equivalent to a mixture of from 30 to 50 weight % of air and from 70 to 50 weight % of one or more inert gases at a temperature from 800°C to 1100°C for a period of time from 5 to 40, preferably from 10 to 25, most preferably from 15 to 20 hours; and
(iii) cooling the resulting stainless steel to room temperature at a rate so as not to damage the surface on the stainless steel.

Inert gases are known to those skilled in the art and include helium, neon, argon and nitrogen, preferably nitrogen or argon.

Preferably the oxidizing environment in step (ii) of the process comprises 40 to 50 weight % of air and the balance one or more inert gases, preferably nitrogen, argon or mixtures thereof.

In step (iii) of the process the cooling rate for the treated stainless steel should be such to prevent spalling of the treated surface. Typically the treated stainless steel may be cooled at a rate of less than 200°C per hour.

Other methods for providing the surface of the present invention will be apparent to those skilled in the art. For example the stainless steel could be treated with an appropriate coating process for example as disclosed in U.S. patent 3,864,093.

Without wishing to be bound by theory it is believed that there may be other layers beneath the chromia such as silica or manganese oxides. It is believed that during the treatment of the steel the chromium from the surface of the steel initially forms a chromia layer, subsequently, the chromium and maganese from the steel may migrate through the chromia layer and form the spinel as the overcoating.

The stainless steel is formed into a part and the surface may be cold worked during or after formation of the part (e.g. boring, honing, shot peening or extrusion), and then the appropriate surface is treated. The steel may be forged, rolled or cast. In one embodiment of the invention the steel is in the form of pipes or tubes. The tubes have an internal surface in accordance with the present invention. These tubes may be used in petrochemical processes such as cracking of hydrocarbons and in particular the cracking of ethane, propane, butane naphtha, gas oil or mixtures thereof. The stainless steel may be in the form of a reactor or vessel having an interior surface in accordance with the present invention. The stainless steel may be in the form of a heat exchanger in which either or both of the internal and/or external surfaces are in accordance with the present invention. Such heat exchangers may be used to control the enthalpy of a fluid passing in or over the heat exchanger.

A particularly useful application for the surfaces of the present invention is in furnace tubes or pipes used for the cracking of alkanes (e.g. ethane, propane, butane, naphtha or mixtures thereof) to olefins (e.g. ethylene, propylene, butene, etc.). Generally in such an operation a feedstock (e.g. ethane) is fed in a gaseous form to a tube, typically having an outside diameter ranging from 1.5 to 8 inches (38.1 to 203.2 mm), e.g. typical outside diameters are 2 inches about 5 cm; 3 inches about 7.6 cm; 3.5 inches about 8.9 cm; 6 inches about 15.2 cm and 7 inches about 20 cm. The tube or pipe runs through a furnace generally maintained at a temperature from about 900°C to 1050°C and the outlet gas generally has a temperature from about 800°C to 900°C. As the feedstock passes through the furnace it releases hydrogen (and other byproducts) and becomes unsaturated (e.g. ethylene). The typical operating conditions such as temperature, pressure and flow rates for such processes are well known to those skilled in the art.

The present invention will now be illustrated by the following nonlimiting examples. In the examples unless otherwise stated parts is parts by weight (e.g. grams) and percent is weight percent

### EXAMPLES

### Example 1

**Sample Preparation**: Sample preparation is from a commercially specified furnace tubes having a composition of the present invention with a bulk chromium content of about 33% (by weight) and manganese of about 1% (by weight). The sample was then heated in an oven up to 1000°C in a reducing atmosphere and maintained at 1000°C for about 16 hours in an atmosphere of a mixture of nitrogen and air, then cooled back down to room temperature.

Metallographic analysis of specimens was carried out by conventional techniques used for characterizing damage-sensitive oxide scales on steels as known to those versed in the art.

Surface structural and chemical analysis was carried out using Scanning Electron Microscopy equipped with light-element Energy Dispersive Spectroscopy (SEM/EDS, Hitachi S-2500), a high resolution field-emission SEM also with light element capability (FESEM-EDS, Hitachi S-4500), Scanning Auger Microprobe (SAM, PHI 600) and Time-of-Flight Secondary Ion Mass Spectrometry (Cameca TOF-SIMS IV).

Figure 1 and 2 are FESEM micrographs of these samples and Figure 3 is a typical metallographic cross-section.

### Example 2

**Sample Preparation**: Coupons from the inlet and outlet of the commercially treated tube were used. Additionally, the same alloy was treated in a comparable manner using laboratory equipment.

Figure 4 shows an EDS spectrum of the laboratory pretreated coupon. Table 1 shows the elemental concentration on the surface of treated alloy coupon or coils. The results in column two are from coupons that were cut out of a commercial tube and treated in the laboratory. Columns three and four show the results of the pretreated commercial coil of Example 1. The results show very good agreement in the capability of the process to increase the content of Mn and Cr on the surface tremendously and decrease nickel content significantly. Also, the content of iron was reduced to a level which was not detectable by the analytical tool that was used.

**TABLE 1**

| **EDS Results of Treated Alloy** | | | |
|---|---|---|---|
| **Element** | **Laboratory Treatment Results** | **Commercial Plant Treatment Results (Coil Inlet)** | **Commercial Plant Treatment Results (Coil Outlet)** |
| O | 4.0 | 6.0 | 6.3 |
| AI | 0.0 | 0.0 | 0.0 |
| Si | 0.4 | 1.7 | 2.7 |
| Ca | 0.0 | 0.3 | 0.5 |
| Cr | 48.0 | 47.2 | 44.6 |
| Mn | 45.7 | 42.5 | 44.2 |
| Fe | 0.0 | 0.0 | 0.0 |
| Ni | 1.9 | 2.3 | 1.8 |
| Nb | 0.0 | 0.0 | 0.0 |

### Example 3

Chromia (Cr₂O₃) powder (≥98% purity) was obtained from SIGMA-ALDRICH. The spinel MnCr₂O₄ powder was manufactured in-house to a purity of ≥98% and its structure confirmed by x-ray diffraction. X-ray Diffraction analysis was carried out using a Siemens D5000 unit with a Cu x-ray source using a 40KV accelerating voltage and a current of 30 ma (shown as Figure 5 for chromia). Crystal structure analysis and assignment was carried out using a Bruker DiffracPlus software package and a PDF-1 database.

Thermal stability analysis was carried out in a controlled atmosphere furnace in the temperature range of 950 to 1150°C with temperature calibrated to ±2°C and controlled to ±0.1 °C. The atmosphere investigated was selected from conditions of vacuum (~10⁻³ torr), or an argon (>99.999% purity) atmosphere, or an argon-5% hydrogen atmosphere, and maintaining a dynamic pressure of 200 mtorr, 1-2 torr or 800 torr. Run times for the study ranged from 4 hours to 300 hours. The conditions selected for the majority of the work at longer run-times were 1-2 torr argon and time steps of 100 hours. The pure powder reference samples were mechanically blended with high purity graphite and placed in a ceramic crucible with a graphite overlayer to approximate an effective carbon activity of approximately one (a_{c} ≅ 1). The stainless steel samples with the current invention of a spinel overcoating were painted with a graphite paste and then placed in a ceramic crucible and covered with graphite to approximate unit carbon activity.

The results for chromia show that the carbide Cr₇C₃ was first detected under 100 hours at 950°C, and formation of the carbide Cr₃C₂ was first observed after 100 hours of 975°C.

In similar experiments with the spinel powder and the spinel overcoating of the present invention, carbide formation was not detected for temperatures of at least 25°C higher.

### Example 4

During the cracking of ethane, coke is formed or laid down, in both the coils and the transfer line exchangers (TLEs) commonly referred to as quench exchangers. As the thickness of the coke builds up, there is an increase in the pressure drop through both the furnace coils and the quench exchangers. Eventually the rise in pressure drop, either in the coils or in the quench exchangers, requires the feed to the furnace to be removed and the furnace decoked. The criteria for decoking the commercial furnaces in this example is either a coil pressure drop of 200 kPa or a TLE pressure drop of 175 kPa, which ever occurs first. The commercial furnace performance is illustrated in the following two figures.

Figure 6 provides the pressure drop through the coils of a typical furnace (H-151) for nine cycles or run times. The typical furnace (H-151) shows that at start of run, the coil pressure drop is about 85 kPa. The coil pressure drop increases to between 120 kPa and 140 kPa prior to being decoked which indicates that furnace H-151 was not decoked due to a rise in coil pressure drop. When the furnace feed is removed and the furnace effluent switched to the decoke system, there is a rise in the coil pressure drop to over 200 kPa. Also shown is the coil pressure drop for a furnace (H-141) in which new coils, with the surface claimed in this patent, have been installed. The graph illustrates that the rate of increase in coil pressure drop was significantly lower then a typical furnace. The graph also shows that the furnace was not decoked during the four hundred days (it was decoked after a run time of 413 days). The small variation in pressure drops are due to the fact that in a commercial furnace and plant, there are changes to system pressures caused by changing ambient temperatures and plant feed rates.

Figure 7 provides the pressure drop through the quench exchangers (TLEs) for the same two furnaces. The typical furnace (H-151) shows that the typical start of run is about 65 kPa and that the pressure drop increase fairly quickly to over 100 kPa, then the rate of increase is much faster as tubes in the quench exchanger become blocked with coke. The graph clearly illustrates that the ability to fully decoke or remove all the coke from the quench exchanger by decoking the furnace is limited and that eventually a typical furnace needs to be shut down and the quench exchangers mechanically cleaned. Furnace H-141 graph illustrates very little coke build up in the quench exchanger for the first 200 days and then a gradual increase to over 125 kPa. The reason that the rate of pressure drop increase was much more gradual is that the nature of the fouling was different. Typically the coke build up is at the inlet to the quench exchangers and results in fully blocked quench exchanger tubes. With the significant reduction in the amount of coke made in the coils and the quench exchanger, H-141 TLEs slowly fouled by small pieces of coke being deposited through out the length of the tubes of the quench exchangers and not at the inlet.

### INDUSTRIAL APPLICABILITY

The present invention provides a process for preparing a surface on stainless steel which is resistant to coking.

## Claims

1. A layered surface having a thickness of from 7 to 25 microns on a stainless steel substrate comprising at least 20 weight % of chromium, 25 to 50 weight % of Ni, less than 1 weight % of niobium, from 1.0 to 2.5 weight % of Mn, less than 1.5 weight % of silicon less than 3 weight % of titanium and all other trace metals, and carbon in an amount less than 0.75 weight %, said surface comprising an outermost layer and at least one layer intermediate the outermost layer and the substrate, said at least one layer intermediate the outermost layer and the substrate having a thickness from 5 to 20 microns comprising not less than 80 weight % of chromia of the formula Cr₂O₃ and said outermost layer having a thickness from 2 to 5 microns comprising not less than 80 weight % of a spinel of the formula MnₓCr₃₋ₓO₄ wherein x is from 0.5 to 2 and covering not less than 100% of the geometrical area defined by said at least one layer intermediate the outermost layer and the substrate.

2. The layered surface according to claim 1, wherein the substrate comprises from 20 to 50 weight % of chromium.

3. The layered surface according to claim 2, wherein the substrate comprises from 1 to 2 weight % of manganese.

4. The layered surface according to claim 3, wherein the substrate comprises from 20 to 38 weight % of chromium.

5. The layered surface according to claim 4, wherein the substrate comprises less than 0.9 weight % of niobium.

6. The layered surface according to claim 5, wherein the substrate comprises less than 1.4 weight % of silicon.

7. The layered surface according to claim 6, wherein the surface area of the outermost layer is at least 50% greater than the surface area of the stainless steel.

8. The layered surface according to claim 7, wherein the stainless steel has been cold worked.

9. The layered surface according to claim 8, wherein the outermost layer comprises not less than 95 weight % of said spinel.

10. The layered surface according to claim 9, wherein the outermost layer is a spinel of the formula MnₓCr₃₋ₓO₄ wherein x is from 0.8 to 1.2.

11. A process for treating a stainless steel comprising comprising at least 20 weight % of chromium, 25 to 50 weight % of Ni, less than 1 weight % of niobium, from 1.0 to 2.5 weight % of Mn, less than 1.5 weight % of silicon less than 3 weight % of titanium and all other trace metals, and carbon in an amount less than 0.75 weight %, which process comprises: (i) heating the stainless steel in a reducing atmosphere comprising from 50 to 100 weight % of hydrogen and from 0 to 50 weight % of one or more Inert gases at rate of 100°C to 150°C per hour to a temperature from 800°C to 1100°C:
(ii) then subjecting the stainless steel to an oxidizing environment having an oxidizing potential equivalent to a mixture of from 30 to 50 weight % of air and from 70 to 50 weight % of one or more inert gases at a temperature from 800°C to 1100°C for a period of time from 5 to 40 hours; and
(iii) cooling the resulting stainless steel to room temperature at a rate so as not to damage the surface on the stainless steel.

12. The process according to claim 11, wherein the stainless steel comprises from 1 to 2 weight % of manganese.

13. The process according to claim 12, wherein the stainless steel comprises from 20 to 38 weight % of chromium.

14. The process according to claim 13, wherein the stainless steel comprises less than 0.9 weight % of niobium.

15. The process according to claim 14, wherein the stainless steel comprises less than 1.4 weight % of silicon.

16. The process according to claim 15, wherein the surface area of the spinel is at least 50% greater than the surface area of the stainless steel.

17. The process according to claim 16, wherein in step (i) the reducing atmosphere comprises 60 to 100 weight % of hydrogen and 0 to 40 weight % of one or more inert gases.

18. The process according to claim 17, wherein in step (ii) the oxidizing environment comprises 40 to 50 weight % of air and the balance one or more inert gases selected from the group consisting of nitrogen and argon.

19. The process according to clam 18, wherein in step (i) the rate of temperature increase is from 120°C to 150°C per hour.

20. The process according to claim 19, wherein in step (iii) the rate of cooling is less than 200°C per hour. ,

21. The process according to claim 20, wherein in step (ii) the time is from 10 to 25 hours.

22. The process according to claim 21, wherein the stainless steel has been cold worked.

23. The process according to claim 22, wherein in step (ii) the time is from 15 to 20 hours.

## Patentansprüche

1. Geschichtete Oberfläche mit einer Dicke von 7 bis 25 µm auf einem Edelstahlsubstrat, die zumindest 20 Gew.-% Chrom, 25 bis 50 Gew.-% Ni, weniger als 1 Gew.-% Niob, 1,0 bis 2,5 Gew.-% Mn, weniger als 1,5 Gew.-% Silicium, weniger als 3 Gew.-% Titan und sämtliche andere Spurenmetalle sowie Kohlenstoff in einer Menge von weniger als 0,75 Gew.-% umfasst, wobei die Oberfläche eine äußerste Schicht und zumindest eine Schicht zwischen äußerster Schicht und dem Substrat umfasst, wobei die zumindest eine Schicht zwischen äußerster Schicht und dem Substrat mit einer Dicke von 5 bis 20 µm nicht weniger als 80 Gew.-% Chromoxid der Formel Cr₂O₃ umfasst und die äußerste Schicht mit einer Dicke von 2 bis 5 µm nicht weniger als 80 Gew.-% eines Spinells der Formel MnₓCr₃₋ₓO₄ umfasst, worin x = 0,5 bis 2 ist, und nicht weniger als 100 % der geometrischen Fläche bedeckt, die durch die zumindest eine Schicht zwischen äußerster Schicht und dem Substrat definiert ist.

2. Geschichtete Oberfläche nach Anspruch 1, worin das Substrat 20 bis 50 Gew.-% Chrom umfasst.

3. Geschichtete Oberfläche nach Anspruch 2, worin das Substrat 1 bis 2 Gew.-% Mangan umfasst.

4. Geschichtete Oberfläche nach Anspruch 3, worin das Substrat 20 bis 38 Gew.-% Chrom umfasst.

5. Geschichtete Oberfläche nach Anspruch 4, worin das Substrat weniger als 0,9 Gew.-% Niob umfasst.

6. Geschichtete Oberfläche nach Anspruch 5, worin das Substrat weniger als 1,4 Gew.-% Silicium umfasst.

7. Geschichtete Oberfläche nach Anspruch 6, worin die Oberfläche der äußersten Schicht zumindest 50 % größer als die Oberfläche des Edelstahls ist.

8. Geschichtete Oberfläche nach Anspruch 7, worin der Edelstahl kaltverarbeitet wurde.

9. Geschichtete Oberfläche nach Anspruch 8, worin die äußerste Schicht nicht weniger als 95 Gew.-% des Spinells umfasst.

10. Geschichtete Oberfläche nach Anspruch 9, worin die äußerste Schicht ein Spinell der Formel MnₓCr₃₋ₓO₄ ist, worin x = 0,8 bis 1,2 ist.

11. Verfahren zur Behandlung von Edelstahl, der zumindest 20 Gew.-% Chrom, 25 bis 50 Gew.-% Ni, weniger als 1 Gew.-% Niob, 1,0 bis 2,5 Gew.-% Mn, weniger als 1,5 Gew.-% Silicium, weniger als 3 Gew.-% Titan und sämtliche andere Spurenmetalle sowie Kohlenstoff in einer Menge von weniger als 0,75 Gew.-% umfasst, wobei das Verfahren Folgendes umfasst:
(i) Erhitzen des Edelstahls in einer reduzierenden Atmosphäre, die 50 bis 100 Gew.-% Wasserstoff und 0 bis 50 Gew.-% eines oder mehrerer Inertgase umfasst, mit einer Geschwindigkeit von 100 °C bis 150 °C pro Stunde auf eine Temperatur von 800 bis 1.100 °C;
(ii) Aussetzen des Edelstahls gegenüber einer oxidierenden Umgebung mit einem Oxidationspotenzial, das einem Gemisch aus 30 bis 50 Gew.-% Luft und 70 bis 50 Gew.-% eines oder mehrerer Inertgase entspricht, bei einer Temperatur von 800 bis 1.100 °C über einen Zeitraum von 5 bis 40 Stunden; und
(iii) Abkühlen des resultierenden Edelstahls auf Raumtemperatur mit einer Geschwindigkeit, die so gewählt ist, dass die Edelstahloberfläche dabei nicht beschädigt wird.

12. Verfahren nach Anspruch 11, worin der Edelstahl 1 bis 2 Gew.-% Mangan umfasst.

13. Verfahren nach Anspruch 12, worin der Edelstahl 20 bis 38 Gew.-% Chrom umfasst.

14. Verfahren nach Anspruch 13, worin der Edelstahl weniger als 0,9 Gew.-% Niob umfasst.

15. Verfahren nach Anspruch 14, worin der Edelstahl weniger als 1,4 Gew.-% Silicium umfasst.

16. Verfahren nach Anspruch 15, worin die Oberfläche des Spinells zumindest 50 % größer als die Oberfläche des Edelstahls ist.

17. Verfahren nach Anspruch 16, worin die reduzierende Atmosphäre in Schritt (i) 60 bis 100 Gew.-% Wasserstoff und 0 bis 40 Gew.-% eines oder mehrerer Inertgase umfasst.

18. Verfahren nach Anspruch 17, worin die oxidierende Umgebung in Schritt (ii) 40 bis 50 Gew.-% Luft und den Rest eines oder mehrer Inertgase umfasst, die aus der aus Stickstoff und Argon bestehenden Gruppe ausgewählt sind.

19. Verfahren nach Anspruch 18, worin die Geschwindigkeit der Temperaturerhöhung in Schritt (i) 120 °C bis 150 °C pro Stunde beträgt.

20. Verfahren nach Anspruch 19, worin in Schritt (iii) die Abkühlungsgeschwindigkeit weniger als 200 °C pro Stunde beträgt.

21. Verfahren nach Anspruch 20, worin die Zeitdauer in Schritt (ii) 10 bis 25 Stunden beträgt.

22. Verfahren nach Anspruch 21, worin der Edelstahl kaltverarbeitet wurde.

23. Verfahren nach Anspruch 22, worin die Zeitdauer in Schritt (ii) 15 bis 20 Stunden beträgt.

## Revendications

1. Surface en couches ayant une épaisseur de 7 à 25 microns sur un substrat d'acier inoxydable comprenant au moins 20% en poids de chrome, 25 à 50% en poids de Ni, moins de 1% en poids de niobium, de 1,0 à 2,5 % en poids de Mn, moins de 1 ,5% en poids de silicium, moins de 3% en poids de titane et tous les autres oligoéléments et du carbone en une quantité inférieure à 0,75% en poids, ladite surface comprenant une couche tout à fait externe et au moins une couche intermédiaire entre la couche tout à fait externe et le substrat, ladite au moins une couche intermédiaire entre la couche tout à fait externe et le substrat ayant une épaisseur de 50 à 20 microns, ne comprenant pas moins de 80% en poids d'oxyde de chrome de la formule Cr₂O₃ et ladite couche tout à fait externe ayant une épaisseur de 2 à 5 microns ne comprenant pas moins de 80% en poids d'un spinelle de la formule MnₓCr₃₋ₓO₄ où x est de 0,5 à 2 et ne couvrant pas moins de 100% de l'aire géométrique définie par ladite au moins une couche entre la couche la plus externe et le substrat.

2. Surface en couches selon la revendication 1, où le substrat comprend 20 à 50% de chrome.

3. Surface en couches selon la revendication 2, où le substrat comprend de 1 à 2% en poids de manganèse.

4. Surface en couche s de la revendication 3, où le substrat comprend de 20 à 38% en poids de chrome.

5. Surface en couches selon la revendication 4, où le substrat comprend moins de 0,9% en poids de niobium.

6. Surface en couches selon la revendication 5, où le substrat comprend moins de 1,4% en poids de silicium.

7. Surface en couche s selon la revendication 6, où l'aire superficielle de la couche tout à fait externe est d'au moins 50% plus importante que l'aire superficielle de l'acier inoxydable.

8. Surface en couche s selon la revendication 7, où ledit acier inoxydable a été laminé à froid.

9. Surface en couches selon la revendication 8, où la couche tout à fait externe ne comprend pas moins de 95% en poids dudit spinelle.

10. Surface en couches selon la revendication 9, où la couche tout à fait externe est un spinelle de formule Mnₓ Cr₃₋ₓO₄ où x est de 0, 8 à 1,2.

11. Procédé de traitement d'un acier inoxydable comprenant au moins 20% en poids de chrome, 25 à 50% en poids de Ni, moins de 1% en poids de niobium, de 1,0 à 2,5% en poids de Mn, moins de 1,5% en poids de silicium, moins de 3% en poids de titane et tous les autres oligoéléments, et du carbone en une quantité inférieure à 0,75% en poids, lequel procédé comprend: (i) chauffer dudit a cier inoxydable dans une atmosphère réductrice comprenant de 50 à 100% en poids d'hydrogène et de 0 à 50% en poids d'un ou plusieurs gaz inertes à raison de 100°C à 150°C par heure jusqu'à une température de 800 à 1100°C;
(ii) puis soumettre l'acier inoxy dable à un environnement oxydant ayant un potentiel oxydant équivalent à un mélange de 30 à 50% en poids d'air et de 70 à 50% en poids d'un ou plusieurs gaz inertes à une température de 800°C à 1100°C pendant une période de temps de 5 à 40 heures; et
(iii)refroidir l'acier inoxydable résultant à température ambiante de façon à ne pas endommager la surface sur l'acier inoxydable.

12. Procédé selon la revendication 11, où l'acier inoxydable comprend 1 à 2% en poids de manganèse.

13. Procédé selon la revendication 12, où l'acier inoxydable comprend de 20 à 38% en poids de chrome.

14. Procédé selon la revendication 13, où l'acier inoxydable comprend moins de 0,9% en poids de niobium.

15. Procédé selon la revendication 14, où l'acier inoxydable comprend moins de 1,4% en poids de silicium.

16. Procédé selon la revendication 14, où l'aire superficielle du spinel les est plus importante d'au moins 50% que l'aire superficielle de l'acier inoxydable.

17. Procédé selon la revendication 16, où à l'étape (i), l'atmosphère réductrice comprend 60 à 100% en poids d'hydrogène et 0 à 40% en poids d'un ou plusieurs gaz inertes.

18. Procédé selon la revendication 17, où à l'étape (ii), l'environnement oxydant comprend 40 à 50% en poids d'air et le reste un ou plusieurs gaz inertes sélectionnés dans le groupe consistant en azote et argon.

19. Procédé selon la revendication 18, où, à l'étape (i), la vitesse d'augmentation de température est de 120 à 150°C par heure.

20. Procédé selon la revendication 19, où, à l'étape (iii), la vitesse de refroidissement est de moins de 200°C par heure.

21. Procédé selon la revendication 20, où, à l'étape (ii), le temps est de 10 à 25 heures.

22. Procédé selon la revendication 21, où, l'acier inoxydable a été laminé à froid.

23. Procédé selon la revendication 22, où, à l'étape (ii), le temps est de 15 à 20 heures.
